# EUROPEAN PATENT SPECIFICATION

(11) **EP 0 531 281 B1**
(45) Date of publication and mention of the grant of the patent: **13.07.1994**
(21) Application number: 90907699.4
(22) Date of filing: 24.05.1990
(51) Int. Cl.: H01F 41/02

(54) **METHOD OF PRODUCING PERMANENT MAGNETS BY POLAR ANISOTROPIC ORIENTATION MOLDING**
VERFAHREN ZUR HERSTELLUNG VON PERMANENTMAGNETEN DURCH POLARE ANISOTROPISCHE ORIENTIERUNGSFORMUNG
PROCEDE DE PRODUCTION D'AIMANTS PERMANENTS PAR MOULAGE A ORIENTATION ANISOTROPE POLAIRE

(43) Date of publication of application: 17.03.1993
(73) Proprietor: EASTMAN KODAK COMPANY, Rochester, New York 14650-2201 (US)
(72) Inventor: LEE, J., Kelly, Rochester, NY 14618 (US); FURLANI, Edward, P., Lancaster, NY 14086 (US); VIGODA, Abraham, M., Rochester, NY 14618 (US)
(74) Representative: Buff, Michel
(86) International application number: US9002755
(87) International publication number: WO9118405

(56) References cited:
- CH-A- 428 967
- FR-A- 1 169 708
- PATENT ABSTRACTS OFJAPAN, Vol. 9, No. 19 (E-292)(1742) 25 January 1985, & JP-A-59 168620
- PATENT ABSTRACTS OF JAPAN, Vol. 9, No. 89 (E-309)(1812) 18 April 1985, & JP-A-59 220911
- PATENT ABSTRACTS OF JAPAN, Vol. 12, No. 158 (E-608)(3005) 13 May 1988, & JP-A-62 271408
- PATENT ABSTRACTS OF JAPAN, Vol. 12, No. 124 (E-601)(2971) 16 April 1988, & JP-A-62 250621

## Description

### Technical Field of the Invention

The present invention relates to a method for producing permanent magnets by molding a plastic material containing a ferromagnetic powder in the presence of a magnetic field, and more particularly to an improved method of performing polar anisotropic orientation molding in orientation magnetic field equipment.

### Background of the Invention

Bonded cylindrical magnets having a plurality of N and S poles arranged alternately and extending parallel to the cylinder axis are employed in such diverse applications as rotors for electric motors and magnetic brushes for handling magnetic toner carrier particles in electrographic copiers. Figure 2 shows such a cylindrical magnet 10 having alternating N, S pole faces 11 extending parallel to the cylindrical axis of the magnet. The magnetic flux lines 12 internal to the magnet enter the body of the magnet at the S poles, extend into the body, and emerge at the N poles.
U.S. Patent No. 4,678,616 issued July 7, 1978 to Kawashima notes that it is known to produce such cylindrical plastic magnets by polar anisotropic orientation molding in orientation magnetic field equipment. However, Kawashima points out that in performing polar anisotropic orientation molding, in orientation magnetic field equipment, it is disadvantageous in that the mold is complicated in structure, and due to the high temperature of the molding process, the electromagnetic coils employed in generating the magnetic field are not stable.

### Summary of the Invention

It is the object of the present invention to provide an improved method of producing long cylindrical magnets by polar anisotropic orientation molding.

In order to achieve the above mentioned object a method according to claim 1 has been developed.

### Brief Description of the Drawings

FIG. 1 is a cross section of a mold for performing polar anisotropic orientation molding according to the present invention;
FIG. 2 is a schematic diagram of a cylindrical magnet having polar anisotropic orientation;
FIG. 3 is a partial cross section showing an area in the region of a pole tip of the mold of FIG. 1;
FIG. 4 is a cross section of a mold having a known configuration;
FIG. 5 is a cross sectional schematic of the mold cavity of FIG. 1 illustrating an alternative known method of molding in a sleeve; and
FIGS. 6 and 7 are plots showing the strength of the magnetic field measured at the surface of magnets produced according to the present invention.

### Modes of Carrying Out the Invention

FIG. 1 is a cross sectional view of a mold employed to carry out the polar anisotropic orientation molding method of the present invention. The mold, generally designated 14, comprises a frame 16 having a top half 16' and a bottom half 16''. The mold parts along line 17 in FIG. 1. The frame 16 is made of high magnetic permeability material such as low carbon steel, and holds 6 radially arranged long thin bars 18. The bars 18 form the pole pieces of an electromagnet, and are wound with conductor coils 20, such as 10 to 30 turns of 8 to 12 guage copper wire with high temperature insulation (e.g. 220°C). One edge of each bar 18 and 24 defines a portion of a cylindrical mold cavity 22. Alternating with the bars 18 of high permeability magnetic material, are bars 24 of low permeability material such as non-magnetic stainless steel or brass.

FIG. 3 shows a partial section of one of the bars 18 at the pole tip. The pole tip 26 is narrowed to concentrate the magnetic field at the tip. The spaces between the pole tips 26 at the surface of the mold cavity are filled with the low magnetic permeability material 24, thereby preventing a magnetic short circuit between the pole tips, and causing the magnetic field to penetrate deeply into the mold cavity 22.

The coils 20 around the pole pieces 18 are connected so that the pole tips 26 alternate in polarity
between N and S, and generating magnetic field lines as shown by lines 28 in FIG. 1.

For most applications, it is required that the poles be evenly spaced around the periphery of the mold cavity. It can be appreciated however that the spacing of the poles may easily be arranged to provide an asymmetrical pattern if desired.

As can be seen from FIG. 1, the construction of the mold is relatively simple, employing a number of identical long thin bars that are inserted into slots in the frame 16.

The mold can be cooled with chilled water through pipes 29 flowing through channels (not shown) inside the mold.

It has been discovered by the present inventors that the magnetic orientation of the particles in the molten binder in the mold takes place in a relatively short time with respect to the mold cycle time. It has been found that with the water cooling and relatively short magnetization cycle time, the coils 20 can be driven with very high currents without encountering any deterioration of the coils due to overheating.

A large (3-6 K watt) direct current power source (not shown) supplies current to the coils 20 in the mold. Preferably the coils in the mold are impedance matched to the power source. A current of between 100 to 600 amps is typically applied for several seconds to form a cylindrical magnet approximately 30 cm long by 3 cm in diameter. For smaller magnets, such as those employed in miniature motors, the time may be reduced to a fraction of a second.

One or more ejector pins 30 may be provided in the center of the pole pieces, as shown in FIG. 1, or alternatively between the coils through the low permeability material 24.

In operation, power is applied to the coils 20 slightly before injecting the molten material into the mold cavity through one or more gates (not shown) at one end of the mold. This allows the full magnetic field strength to be established prior to introducing the molten material into the mold. Typical nozzle temperatures for injecting nylon or similar polymer binder heavily loaded with anisotropic ferromagnetic powder such as barium ferrite into the mold are 250° to 290°C. After several seconds, current to the coils 20 is terminated. After a sufficient cooling period (15 seconds to 2 minutes depending on the size of the part), the mold is opened and the magnet is removed. Although the process has been found to produce magnets having sufficient strength that no further magnetization is required, post molding magnetization employing a fixture similar to the mold itself can be performed, and will provide a marginal increase in the external magnetic field of the magnet. Such a fixture may be connected to a capacitor discharge magnetizer which provides several thousands of amps for a small fraction of a second.

FIG. 4 shows a known way of constructing the mold cavity. In this embodiment, spaces between the tips 24 of the magnetic pole pieces 18 around the mold cavity 22 are occupied by thin walled sections 32 of the material comprising the pole piece. When the current in the coils 20 is sufficiently high, the thin walled sections 32 of the mold cavity will magnetically saturate, thereby causing the magnetic field to extend into the mold cavity as shown by flux lines 34 in FIG. 4. The low carbon steel that is employed in the pole pieces for example saturates at 19,000 Gauss, which is readily achieved with the arrangement described.

The pole pieces and mold cavity shown in FIG. 4 can be readily produced using the technique of wire electro-discharge machining (EDM).

According to another known way, as illustrated in FIG. 5, the cylindrical magnets may be formed by molding inside a thin walled tube 36, such as non-magnetic stainless steel. Although non-magnetic stainless steel is presently preferred for the tube, other materials may be employed, such as low carbon steel or brass. In this embodiment, it is not necessary to provide spacers between the pole tips 26. The tube 36 is inserted into the mold prior to injecting the magnetic material into the mold. It has been found that the molded magnetic roller is easily removed from the tube 36 after cooling. Different size magnets over a limited range, can be produced in the same mold by varying the thickness of the tube.

The relative width of the pole tips 26 determines the strength of the magnetic field produced at the surface of the magnets. The narrower the pole tips, the more concentrated the magnetic field, and hence the higher the magnetisation produced. FIG. 6 is a plot showing the magnetic field measured around the circumference of a magnetic roller produced in a mold having wide pole tips (e.g. slightly less than 60°). FIG. 7 is a similar plot showing the increased magnetic field intensity resulting from a mold having narrowed pole tips as shown in FIG. 1. As can be seen by comparing FIGS. 6 and 7, an increase in field strength of between 20 to 30% was achieved by narrowing the pole tips. Both the broad ple and the narrow pole shape are useful depending on the application.

### Industrial Applicability and Advantages

The magnet molding method according to the present invention is useful for making rotors for electrical motors and magnetic brushes for electrographic printers. The method is advantageous in that magnets exhibiting very strong uniform fields are produced.

## Claims

1. A method of producing a long cylindrical magnet (2) polar anisotropic orientation molding, characterized by:
the mold having electromagnets (20) comprising long thin bars (18) of high permeability magnetic material, wrapped with current conducting coils, one edge of each bar defining a magnetizing pole tip (26) aligned parallel with the cylindrical axis of the mold, and defining portions of the wall of the mold cavity, whereby the magnet is molded in contact with the pole tips (26) of the orienting magnets, thereby increasing the magnetic field strength of the molded magnet.

2. The method of producing a long cylindrical magnet by polar anisotropic orientation molding of Claim 1, characterized by:
portions of the walls of the mold cavity being defined by a plurality of alternating N and S pole tips (26) of the electromagnets (20) employed to orient the magnetic material, and the pole tips (26) being spaced apart by low permeability material (24), whereby the magnetic flux from the pole tips is directed into he cavity of the mold, thereby increasing the magnetic field strength of the molded magnets.

3. The method of producing a long cylindrical magnet by polar anisotropic orientation molding of Claim 1, characterized by:
portions of the walls of the mold cavity being defined by the pole tips (26) of the electromagnets (20) employed in the orientation, and the electromagnets being driven with a large current for a relatively short time during the mold cycle.

4. The method of producing a long cylindrical magnet by polar anisotropic orientation molding of Claim 1, characterized by:
cooling the mold with chilled water during the molding cycle, and driving the electromagnets with a predetermined current for a small fraction of the mold cycle.

## Patentansprüche

1. Verfahren zur Herstellung eines langgestreckten Zylindermagneten (2) durch polarisiertes anisotropes orientierungsformen, **dadurch gekennzeichnet, daß**
die Form mit Elektromagneten (20) versehen ist, die lange, dünne Stäbe (18) umfassen, welche aus hochpermeablem, von stromleitenden Spulen umgebenem magnetischem Material bestehen und deren eine Kante jeweils eine magnetisierende, parallel zur Zylinderachse der Form ausgerichtete Polspitze (26) sowie Oberflächenbereiche der Forminnenfläche bildet, wobei der Magnet während des Formvorgangs in Berührung mit den Polspitzen (26) der Orientierungsmagnete ist und sich dadurch die magnetische Feldstärke des geformten Magneten erhöht.

2. Verfahren nach Anspruch 1, dadurch gekennzeichnet, daß zur Orientierung des Magnetmaterials Oberflächenbereiche der Forminnenfläche aus einer Vielzahl alternierender Nord- und Südpolspitzen (26) der Elektromagnete (20) gebildet werden und daß die Polspitzen (26) durch geringpermeables Material (24) im Abstand voneinander gehalten werden, wodurch der Magnetfluß von den Polspitzen in das Forminnere geleitet wird und sich dadurch die magnetische Feldstärke der geformten Magnete erhöht.

3. Verfahren nach Anspruch 1, dadurch gekennzeichnet, daß Oberflächenbereiche der Forminnenfläche durch die der Orientierung des Magnetmaterials dienenden Polspitzen (26) der Elektromagnete (20) gebildet werden und die Elektromagnete während des Formvorgangs für relativ kurze Zeit mit hoher Stromstärke erregt werden.

4. Verfahren nach Anspruch 1, dadurch gekennzeichnet, daß die Form während des Formvorgangs mit kaltem Wasser gekühlt wird und daß die Elektromagnete während eines Bruchteils des Formvorgangs mit einer vorbestimmten Stromstärke erregt werden.

## Revendications

1. Procédé de Production d'un aimant cylindrique long (2) par moulage à orientation anisotropique polaire, caractérisé par :
le moule comportant des électro-aimants (20) comprenant des barres fines et longues (18) d'un matériau magnétique à haute perméabilité, entourées de bobines conductrices de courant, un bord de chaque barre définissant une pointe de pôle de magnétisation (26) alignée de façon parallèle à l'axe du cylindre du moule et définissant des parties de paroi d'un creux de moule, dans lequel l'aimant est moulé en contact avec les pointes de pôle (26) des aimants d'orientation, augmentant de ce fait l'intensité du champ magnétique de l'aimant moulé.

2. Procédé de production d'un aimant cylindrique long par moulage à orientation anisotropique polaire selon la revendication 1, caractérisé par :
des parties de parois du creux de moule étant définies par une pluralité de pointes de pôle (26), N et S en alternance, des électro-aimants (20) utilisés pour orienter le matériau magnétique ainsi que les pointes de pôle (26) étant séparées par un matériau à faible perméabilité (24), dans lequel le flux magnétique des pointes de pôle est dirigé dans le creux de moule, augmentant de ce fait l'intensité du champ magnétique des aimants moulés.

3. Procédé de production d'un aimant cylindrique long par moulage à orientation anisotropique polaire selon la revendication 1, caractérisé par :
des portions des parois du creux de moule étant définies par les pointes de pôle (26) des électro-aimants (20) utilisés dans l'orientation et les électro-aimants étant commandés avec un courant important pour une durée relativement courte pendant le cycle de moulage.

4. Procédé de production d'un aimant cylindrique long par moulage à orientation anisotropique polaire selon la revendication 1, caractérisé par :
le refroidissement du moule par de l'eau refroidie pendant le cycle de moulage et la commande des électro-aimants par un courant prédéterminé pendant une courte fraction du cycle de moulage.
